# EUROPEAN PATENT SPECIFICATION

(11) **EP 2 643 508 B1**
(45) Date of publication and mention of the grant of the patent: **07.01.2015**
(21) Application number: 11793645.0
(22) Date of filing: 07.11.2011
(51) Int. Cl.: D02G 3/04, D02G 3/44

(54) **FLAME RESISTANT FABRIC FOR PROTECTIVE CLOTHING**
FLAMMHEMMENDER STOFF FÜR SCHUTZKLEIDUNG
TISSU RÉSISTANT À LA FLAMME POUR VÊTEMENTS PROTECTEURS

(30) Priority: 24.11.2010 AT 19532010
(43) Date of publication of application: 02.10.2013
(73) Proprietor: Lenzing AG, 4860 Lenzing (AT)
(72) Inventor: GSTETTNER, Alexander, 4663 Laakirchen (AT); BURROW, Tom, Derby DE73 6NJ (GB); MATHES, Ulf, 4690 Schwanenstadt (AT)
(74) Representative: Hanemann, Otto
(86) International application number: PCT/AT2011/000448
(87) International publication number: WO 2012/068600

(56) References cited:
- WO-A2-2009/012266
- AT-A4- 508 653
- DE-A1- 3 307 449
- US-A1- 2005 025 962
- US-A1- 2005 032 449
- US-A1- 2006 292 953
- US-A1- 2011 191 949

## Description

### Field of application

A new flame resistant fabric has been invented that uses the properties of known flame resistant fibres combined with non-flame resistant fibres to produce a fabric with exceptional resistance to flame, surprising physical properties and enhanced comfort to the user compared to other flame resistant fabrics.

"Flame resistance" is a characteristic of a material such as a fibre or fabric that does not burn in a normal air atmosphere. When exposed to a flame, it will not support combustion when the flame is removed. "Flame resistance" should not be confused with "flame retardant" which is a term used to describe a chemical substance that imparts flame resistance to fabric. Flame retardant is also used to describe fabrics which exhibit a reduced rate of burning but may not offer any protection to the user from flames.

It is well known that flame resistant fabrics, especially those made from flame resistant fibres, can be used to give protection against exposure to flame. It is normal practice that firefighters wear garments that will protect the user from flame in a hazardous situation. The garment is expected to prevent direct exposure to flames of the clothed user's skin, thereby reducing the risk of suffering burn injuries.

Other professions where protection from flame is required include police and security personnel, military personnel, and workers in the gas and petroleum industries.

Protective clothing for molten metal splash protection is used by welders and metal industry workers. In the metal industry high levels of energy are used to melt metal and to create electric arcs. Therefore protective clothing is needed to protect against liquid metal splashes and against electric arcs. Utility personnel working on high voltage installations may be exposed to small metal splashes, when electric arc is produced accidentally.

It is highly desirable that fabrics used in these applications should be comfortable to wear, should perform well physically and be aesthetically suited to the task - colour appearance, style and feel.

It is common for workers who use personal protective clothing to be working in a high stress environment with a high work load leading to high physiological energy consumption. This physiological strain leads to generation of body heat and moisture inside the garment. It is highly desirable that fabrics used for the construction of the garments should be capable of dissipating body heat and moisture to prevent over heating (heat stress) of the user's body. Fabrics that allow body heat and moisture to escape produce garments that feel more comfortable to wear and also prolong the working time that can be achieved without exceeding maximum physiological stress levels.

It is well known, that cellulosic fibres can give enhanced comfort compared to synthetic fibres. This is, because cellulosic fibres are hydrophilic and absorb moisture vapour and liquid water. Controlling the movement and distribution of water in the fabric is an inherent property of a cellulosic fibre.

In the intended applications, fabrics are expected to be unaffected by all activities that they are subjected to This means they need to have high tear strength, high abrasion resistance and good resistance to snagging.

Fabrics also need to retain their appearance over a prolonged period of use and care. Therefore fabrics need to be washable and have good washing stability, low shrinkage, good pilling performance, and good colour fastness to washing and light.

It is common for organizations that equip workers with personal protective clothing to require that the clothing conforms to the organisation's corporate colours: There are also many cases where the colour of a garment is important for its function such as black for riot police or high visibility yellow, orange or green for firefighters and industrial workers. Therefore it is highly desirable that fabrics used for these applications can be dyed easily to a wide range of colours and give good fastness performance.

This invention is a flame resistant fabric suitable for use in garments intended to protect workers in the metal industry and the utility industry from accidental exposure to flame, molten metal - except alumina - and electric arcs. The fabric produces garments which are comfortable to wear, have a minimal effect on the physiological performance of the wearer and have excellent physical properties,

### Prior Art

Textile materials vary considerably in their ability to resist flame and hence protect underlying materials. Most fabrics made from natural fibres and from synthetic fibres will burn when exposed to flame. The rate of burn and ease of ignition are determined primarily by the chemical nature of the polymer from which the fibre is made and the construction of the fabric. Many polymers, such as cellulose, polyester and nylon will burn readily. The rate of burn is lower the heavier a fabric is. Wool is the most common natural fibre which has flame resistant properties to some degree - heavy weight wool fabrics will not burn readily and are used in firefighter's clothing historically.

Fabrics for protection against molten metal splash as used in the metal industry including welding application are often extremely heavy and stiff. Fabric weights are ranging from 330 to 600g/m². They are made from materials such as flame resistant treated cotton.

Fabrics can be treated to make them flame resistant by applying an appropriate chemical to the fabric. The first FR treated fabrics used inorganic salts such as aluminium hydroxide, antimony trioxide and borates to make cotton fabrics flame resistant. These were effective but were non-durable to washing.

Organic phosphorous containing compounds that are reacted onto the cotton either by grafting or network formation are more durable and are widely used. Two of the leading brand names are Proban® and Pyrovatex®. While these finishes are durable, they can be removed by harsh chemical treatments and the level of finish reduces with the number of washing cycles. The finish application has an adverse stiffening effect on the fabric. Fabrics of this type are in use for protection from flame, molten metal splash and electric arc. When exposed to flame, molten metal or electric arcs, fabrics of this type will not burn, but become highly embrittled and may break open leaving the wearer's skin exposed to the hazard.

The protection properties of fabrics against liquid iron splashes are classified by a three-stage system: E1 characterizes the lowest resistance while E3 stands for the highest molten iron resistance. For an E3-fabric a fabric weight of at least 450g/m² FR treated Cotton is needed. Common FR treated cotton fabrics of a fabric weight of 290g/m² only shows E1 properties.

The first flame resistant man made fibres produced were made by the viscose process. A high viscosity liquid flame resistant additive was dispersed in the spinning solution prior to extrusion of the fibre. The liquid was trapped in the cellulose by physical means as very small bubbles. The result was effective as a flame resistant fibre, but the additive could be removed by repeated washing. The strength of the fibre is reduced in proportion to the amount of additive included. The additive was withdrawn from the market due to safety concerns and production of the fibre was discontinued.

An improved flame resistant viscose fibre can be produced by using a solid pigment flame retardant. Fibre of this type will be referred to as FR viscose The pigment is finely ground and mixed with the spinning solution prior to extrusion of the fibre. The result is a dispersion of the insoluble particulate additive in the fibre. The strength of the fibre is reduced in proportion to the amount of additive included. All of the cellulose in the fibre contains some of the additive and the additive cannot be removed by washing or normal fabric dyeing or finishing processes. Hence the result of the process is an inherently flame resistant fibre. A well-known fibre of this kind is Visil®, which contains silica pigment flame retardant.

A further improvement can be achieved by incorporating the solid pigment flame retardant in the spinning solution used to produce modal fibre, The modal process is a modified viscose process designed to produce a fibre with a higher strength and higher wet modulus than normal viscose. The resultant fibre containing the flame retardant pigment is inherently flame resistant. It is stronger than fibre produced by the viscose process and gives fabrics with higher strength and better stability. Fibre of this type will be referred to for the purposes of this invention as "FR Modal" but note that the properties of the fibre do not conform to the BISFA (INTERNATIONAL BUREAU FOR THE STANDARDISATION OF MAN-MADE FIBRES) definition of modal fibre. Proven flame retardant pigments for this kind of fibres are organic phosphorous compounds and a preferred pigment is Exolith® (2'-oxybis[5,5-dimethyl-1,3,2-dioxaphosphorinan]2,2'disulfid).

FR Modal is used in 100% form in only a few applications in the field of apparel such as metallised fabrics or fabrics which are mixtures of two or more yarns. On its own its performance is inadequate in a number of respects compared to other products.

In the same way Lyocell fibres can be made flame resistant. Due to the different manufacturing conditions usually different pigments are suitable. Fibre of this type will be referred to as Lyocell FR.

An alternative approach to producing an FR fibre is to modify the polymer from which the fibre is made so that it is inherently flame resistant but can still be formed into a fibre. There are many examples of such fibres but the leading ones being used in personal protective clothing are meta-aramid, para-aramid, Polybenzimidazole (PBI), FR polyester and modacrylic.

Flame resistant fibres can often be used on their own to make fabrics which function well. They can also be used in blends with each other and with non flame resistant fibres to produce fabrics. Such blend fabrics can have properties which are a combination of the properties of the component fibres.

There are many flame resistant fabrics available in the market. The most widely used in personal protective clothing are (blend ratios are given in %w/w): Flame resistant treated 100% cotton; Flame resistant treated cotton / polyamide blend (typ 85/15); Flame resistant treated polyester / cotton blend (typ 50/50); Modacrylic / cotton blend (typ 55/45); Modacrylic / cotton / aramid blend (typ 25/25/50); Modacrylic / lyocell / aramid blend (typ 25/25/50); 100% meta-aramid; Meta-aramid / para-aramid blend (typ 80/20); Meta-aramid / para-aramid/Anti static blend (typ 93/5/2); Meta-aramid / FR Modal blend (typ 70/30); Meta-aramid / FR Modal blend (typ 50/50; Meta-aramid / FR Modal blend (typ 35/65)).

Each of these fabrics has its merits and deficiencies, as can be seen from Table 2 (see Example 2). The fabric selection process used by garment makers and specifiers is based on a judgement of the overall performance and the required level based on risk analysis. None of the fabrics provides all of the criteria of an ideal fabric listed in Table 2.

FR treated cotton and cotton blend fabrics give poor to medium performance, fair comfort, relatively easy processing and are the most affordable. Modacrylic blends give fair performance but poor comfort and cost more. Aramid fabrics give good performance and washing performance but are not comfortable and are expensive. None of the fabrics currently available are rated as good for metal splash or for electric arc. Only the meta-aramid/FR Modal fabric is rated as good for break open behaviour.

Adding FR Modal to an aramid fabric improves its overall performance and reduces the cost.

US 2005/0025962 A1 claims in claim 1 a very broad range of staple fiber blend compositions including aramide fibers, flame retardant cellulosic fibers and polyamide fibers. But in the examples only three-component-yarns with up to 55 % of FR rayon fibers are disclosed.

US 2005/0032449 A1 discloses only up to 35 % FR rayon in the yarns of the examples and generally an FR cellulosic fibre content of 15-50%, preferably 25-40%, is recommended. In a similar way US 2011/0191949 A1 recommends that the FR cellulosic component shall be used only up to 50% in the fabric, preferably from 30-35%.

Each of the currently available fabrics has deficiencies in one or more respects. No single fabric has given good all-round performance, protection, comfort, processability and care properties at a reasonable cost. This is the target of the invention.

### Objective

The objective of this invention is to produce a fabric for use in personal protective clothing which resolves the deficiencies of the prior art described above. It should show excellent performance in terms of safety of the user, especially in respect of metal splash protection, electric arc protection and break open behaviour. It should also be at lower cost and with better comfort and aesthetic properties than current products to ensure that garments made from it have all of the required performance for the intended applications.

Current products in the market perform well in protecting the user, but they are expensive, which means their use is limited. They are made from, at least in part, fibres with poor comfort and aesthetic properties and they can be difficult to produce because of poor dyeability. Currently used fabrics especially for the molten metal industry are stiff and heavy (fabric weights ranging from 330 to 600g/m²). For electrical utilities, insulation against electric arc as well as improved break open performance after electric arc exposure are important safety requirements. There was a need for a fabric which will deliver:
- Protection :
   ∘ Inherently flame resistant for the life of the product
   ∘ Extremely lightweight fabrics providing maximum protection against liquid metal splash
   ∘ Improved break open after electric arc exposure
   ∘ Very good break open behaviour after flame exposure; the fabric remains soft and intact
   ∘ Cool to the touch immediately after exposure to flame
   ∘ Very good insulation against heat and flame
- Mechanical Performance and Durability:
   ∘ High tear resistance
   ∘ Low Pilling
   ∘ Excellent abrasion properties
- Physiological Performance:
   ∘ Good thermal properties giving more efficient cooling of the user,
   ∘ Improved physiological performance of the user
- Comfort:
   ∘ High and rapid moisture absorption
   ∘ Good short-term water absorption capacity
   ∘ Cool touch
- Processability:
   ∘ Fabric can be piece dyed
   ∘ Wide range of colours achievable
   ∘ Fabric printable using vat or reactive dye systems
- Washing Performance :
   ∘ Stable to washing
   ∘ Low washing shrinkage
- Environment / Sustainability :
   ∘ Fibres which are OKOTEX Standard 100
   ∘ Fibres which are highly sustainable

### Description

The product of the invention is a flame resistant fabric for use in personal protective clothing which provides a high level of protection from flames and other sources of heat such as molten metal splash and electric arc, which is made from a yarn which is an intimate blend of FR Modal fibres with high temperature resistant polymer fibres and standard flammable synthetic fibres.

The blend ratio of the yarn is:
from 65 to 90% FR Modal fibres,
from 10 to 20 % high temperature resistant polymer fibres and
from 10 to 20% standard synthetic fibres,
   preferably
from 65 to 75 % FR Modal,
from 12,5 to 17,5 % high temperature resistant polymer fibres and
from 12,5 to 17,5 % standard flammable synthetic fibres.

It is surprising that a fabric with this fibre content can give such exceptional performance. It is generally believed by those skilled in the art that a fabric will have better flammability performance and give better protection the higher the content of aramid fibre. The fabric of the invention contains a high percentage of FR Modal fibre and yet performs better than currently available fabrics made using a high percentage of aramid fibre.

Anti static properties of the fabric can be achieved by adding 1 to 5% antistatic staple fibre to the blend, or by creating an antistatic grid by including in the fabric, yarns consisting of the ground yarn twisted with antistatic continuous filament yarns. All fibres used in the blend can be dope dyed (spun dyed) fibres.

The FR Modal fibre of the yarn has been made flame resistant by addition of an FR agent during or after fibre production.

The high temperature resistant polymer fibres are chosen from the group consisting of para-aramid, meta-aramid, aromatic polyester (PES), PBI and blends of these fibres. Preferably, the high temperature resistant polymer fibres are para-aramid fibres. Fibres can be dope dyed (spun dyed) or stock dyed as staple fibre or top dyed.

The standard flammable synthetic fibres are chosen from the group consisting of polyamid 6 (PA6), polyamid 6 (PA6.6) and polyester (PES) Preferably, the fibres are PA6 and especially preferred is a high-tenacity PA6 fibre. Fibres can be dope dyed (spun dyed) or stock dyed as staple fibre or dyed as tops, yarn or fabric.

More specifically the product of the invention is a fabric consisting of a yarn; which is a blend of FR Modal, and a para-aramid or meta-aramid or a blend of the two aramids and flammable high tenacity PA6. The fabric may be woven, knitted or produced with non-woven technologies.

The woven fabric has a warp and weft composed of the yarn according to the invention.

Even though the fabric includes a percentage of flammable standard synthetic fibres, the fabric has exceptional flammability and protective performance. It will not burn, it does not break open when exposed to a flame and continues to provide a barrier to flame. Furthermore, the fabric provides a high level of molten iron ("metal splash") protection even at a low fabric weight, as well as superior electric arc protection. For good orders sake it should be mentioned that the fabric of the invention does not protect against molten alumina.

Each of the fibres in the blend may be dope dyed (i. e. spun dyed). This will produce a fabric with very high colour fastness. Only very expensive Aramids have been available as dope dyed fibres so far.

The exceptional flammability and protective performance of the fabric of the invention has previously only been possible with significantly heavier, much more expensive fabrics such as PBI, 100% aramid or Lenzing FR/meta-aramid, as well as heavy Modacrylic - or flame resistant treated cotton blends and inorganic based fibres.

All of this is achieved with a fabric that has a lower fabric weight, better protection and lower production cost than other fabrics with similar performance and the fabric is much more comfortable because of the high proportion of cellulosic fibres.

The yarn is produced from staple fibre by spinning the yarn using conventional techniques such as ring spinning, open end spinning, vortex spinning, worsted spinning, semi-worsted spinning or any of the variations on these used in the yarn spinning industry. The staple length of the fibres for the primary yarn may be between 35 mm up to 160 mm. Especially preferred are fibres with a staple length of between 75 and 90 mm. The staple length will need to be appropriate to the spinning system selected. At least the FR Modal fibres in the yarn according to the invention should be of this staple length, but in a preferred embodiment of the invention all fibres in the yarn according to the invention should be of this staple length.

The use of fibres with a staple length of between 75 and 90 mm provides for a high durability of even lightweight fabrics with a low pilling and high tenacity, tear strength and abrasion resistance. At the same time the yarns according to the invention and also the fabrics made of these yarns have a more plain, less hairy appearance.

The linear density (= titre) of the fibres and filaments used in the fabric will be chosen to fit with the intended application. Generally it will be in the range commonly used for such textile applications. The linear density will depend on the yarn spinning system used for the yarn.

During the preparatory processes prior to spinning the FR Modal fibre, the high temperature resistant polymer fibre and the standard flammable synthetic fibres are blended together in the required proportions. The yarn according to the invention is an intimate blend of the three fibres with each of the fibres well dispersed throughout the final yarn. This blending can be done during opening of the fibres, during carding or during drawing of the sliver.

The blend ratio of the yarn according to the invention in an especially preferred embodiment is
70 % FR Modal,
15% high temperature resistant polymer fibres and
15% standard synthetic fibres.

Anti static properties of the fabric can be added by blending 1 to 5% antistatic fibre in or by creating an anti static grid in the fabric using yarns that are made by twisting the ground yarn (according to the invention) with antistatic continuous filament yarns.

The proportion of para-aramid fibre in the yarn may be up to 30%, but the cost of the fabric increases with increasing para-aramid content with no appreciable increase in performance against the applicable standards.

One or more of the individual fibre components in the fabric are dope dyed, stock dyed or dyed tops or can be dyed in the yarn or fabric. The high temperature resistant polymer fibres can be either dope dyed or dyed in flock or tops state. By using 100% dope dyed fibres the fabric colour fastness will be improved while at the same time a cost saving on fabric dyeing can be achieved.

The fabric weight, construction and weave of the woven fabric are selected to deliver a fabric of the style and properties required for the application. E.g. the fabric construction may be a plain weave, twill, hopsack, satin, sateen or any other weave which is appropriate to a protective clothing application. For knitted fabrics a plain jersey, pique or any other suitable fabric construction is possible. The fabric may be a lightweight (i. e. a weight per unit area of 100 to 150 g/m²) plain weave for shirting applications. It may be a medium weight (i. e. a weight per unit area of 150 to 230 g/m²) twill weave for trousers. It may also be a heavyweight (i. e. a weight per unit area of 230 to 350 g/m²) twill weave for jackets and other outerwear. The basic principle of the invention can be incorporated in a wide variety of fabrics. It will work regardless of the weave or construction, provided the correct blends and arrangements of yarns are used. Only exceptionally lightweight fabrics (less than 100 g/m²) would not show the benefits of the invention.

The fabric of the invention may also be produced using a nonwoven fabric production method. Clearly for a nonwoven process a yarn is not required but all what was said above about the nature, properties and treatment of the yarn fibres as well as for the blend ratios applies for the composition of such nonwovens as well. The fibre components are blended together and made into a nonwoven fabric without first spinning a yarn. An example of such a fabric is a needlefelt fabric where the individual fibre components are mixed together in a blending device and then carded, crosslaid and needled to give a fabric. Such a fabric is of use e. g. as an insulating liner in a garment or could be used to make simple garments such as aprons.

### Use of the invention

The product of this invention is intended to be used as one of the primary components of clothing for personal protection in situations where there is a risk of exposure to flame, electric arc and liquid metal splash. The fabric is used to make garments that cover the body of the user to protect the skin from exposure to flames or to other sources of heat such as metal splash - except alumina - and electric arc that would cause injury.

Garments are usually made by assembling cut shaped pieces of fabric by sewing them together. The product of this invention may be the sole fabric used in making a garment or may be one component of a garment; the other components consisting of fabrics of different design and purpose. It may also be combined with other fabrics by laminating prior to cutting the shaped pieces for garment assembly.

The product of this invention may be used as a layer of fabric on the inside of a garment. It may be used as a layer on the outside of a garment or it may be used as an internal component between two or more other fabrics. It may also be used to provide more than one layer in the garment. For example it could be used as the inner layer of the garment and as the outer layer of the garment with a third layer of a flame resistant wadding between the inner and outer layers.

The fabric of the invention may be used for the production of all types of garments where protection from flames is a primary purpose. It can be used for jackets, coats, trousers, shirts, polos, sweaters and jumpers, sweatshirts, T-shirts, socks, aprons, gloves and gauntlets, hoods for head protection other headwear and any other garment that may be worn for the purpose of protecting the wearer from flame and similar hazards. The fabric may also be used in other articles which are intended to provide protection of people or property from exposure to flame such as shoe and boot components, welding screens, fire curtains, tents, sleeping bags, tarpaulins and any other similar articles made in whole or in part from fabric.

Coloured fabrics for the intended applications are preferably achieved by using spun dyed fibres, by piece dyeing or by printing, but in general all dyeing techniques are applicable.

### Example 1

A twill weave fabric was woven from the following components:
- Yarn: A Nm 45/2 worsted spun yarn in which 70% of the fibre was 3.3 dtex Lenzing FR® (1/3 with 75 mm and 2/3 with 90 mm staple length), 15% of the fibre was 1.7 dtex 100 mm staple length para-aramid and 15% of the fibre was high tenacity PA6. Lenzing FR® is an FR modal fibre available from Lenzing AG, Austria, which is produced according to a modal process (see AT-508687) and which contains Exolith® as an incorporated FR pigment. The three fibre components were blended together in drafting of the slivers during preparatory processing.

The fabric warp count was 30 threads per cm. The weft count was 26 threads per cm.

The resulting fabric had a mass per unit area of 260 g/m²

### Flame protection:

The resulting fabric could not be ignited in normal atmospheric conditions. On exposure to flame directed at the surface of the fabric, the fabric charred but maintained its structure and continued to act as a barrier to flame. No holes were formed in the fabric. The fabric remained soft and flexible without any break open after flame exposure according to EN ISO 15025 procedure A (surface ignition). Furthermore no heat shrinkage of the fabric was observed when the flame was directed at the fabric surface and during the whole flaming time of 10 seconds.

Afterflame and afterglow of the fabric when tested according to EN ISO 15025 procedure A were 0 seconds in the warp direction and 0 seconds in the weft direction.

Protective garments - jackets and trousers - were assembled from the fabric and evaluated as follows.

### Testing with an instrumented manikin

according to ISO 13506.3: Protective clothing against heat and flame - Test method for complete garments - Prediction of burn injury using an instrumented manikin. This test method characterizes the thermal protection provided by garments, based on the measurement of heat transfer to a full-size manikin exposed to a laboratory simulation of a fire with controlled heat flux density, duration and flame distribution. The heat transfer measurements can also be used to calculate the predicted skin burn injury resulting from the exposure. Garments made from the fabric according to the invention were compared with garments made from a 100% aramid fabric (Tables 1 and 2).

**Table 1 - Burn prediction:**

| Degree of burns/Total Burns(%) | 1st | 2nd | 3rd |
|---|---|---|---|
| Fabric of the invention: | 7 | 16,7 | 0,9 |
| 100% Aramid: | 5,3 | 18,4 | 10,5 |

**Table 2 - Dimensional Change after flame exposure:**

| Location: (Shrinkage%) | Fabric of Invention | 100% Aramid |
|---|---|---|
| Jacket length | +3,6 | -8 |
| Jacket width | +2,0 | -2,0 |
| Jacket upper arm | -10,9 | n/a* |
| Arm length | +2,1 | -5,0 |
| Trousers length | -1,2 | -16,7 |
| Trousers thigh | -7,9 | n/a* |

| | | |
|---|---|---|
| n/a*: after flame exposure the garment was too brittle for evaluation | | |

The garment made from the fabric of the invention showed far less burns in comparison with 100% Aramid garments. After the flame exposure the garments were removed from the manikin to measure the size and shrinkage of the garment. Parts of the 100% Aramid garments were too brittle to measure - the jacket upper arm and the trouser thigh. The fabric of the invention remained intact in one piece. No severe damage was observed. The fabric remained flexible and did not break open.

Surprisingly, the fabric of the invention does not shrink during the flame exposure. In fact the opposite occurs - some parts of the garment increased in dimensions. The 100% Aramid garment show significant flame shrinkage.

In the visual evaluation of the test garments it can clearly be seen that the garment made from the fabric of the invention is creating a kind of extra protection cushion when exposed to flame.

### Metal splash protection:

The fabric of the invention was tested according to ISO 9185 and classification according to EN ISO 11612. Despite of it's relatively low fabric weight of 260 g/m² the result was on the highest protection level which can be achieved: E3. For comparison: A typical fabric already used for iron metal splash protection has a fabric weight of 400 g/m² and only shows a protection level E1.

This test assesses the ability of the fabric to withstand a certain quantity of molten metal and how the metal interacts with the fabric. The best performing materials retain their structure and the metal does not adhere to the surface. Damage done to the fabric is minimized.

### Electric Arc protection:

The fabric of the invention was tested according to EN ISO IEC 61482 1-2, 4kA and 7kA. The fabric passed with excellent values the required Stoll criteria for 4kA, and exhibited no break open of the fabric in a single layer, when tested to 7kA. The Stoll curve is a curve of thermal energy and time produced from data on human tissue tolerance to heat and used to predict the onset of second-degree burn injury (cited from EN ISO IEC 61482 1-2).

### Mechanical Performance testing:

The tear test results tested according to ISO 13937-2 were as follows compared to some of the other products currently used in personal protective clothing in Table 3:

**Table 3 - Fabric Performance Results**

| Fabric | Fabric weight (g/m²) | Warp tear strength | Weft tear strength | Heat penetration coefficient Alambeta | Short time Water vapour absorption [Fi] | Colour Fastness |
|---|---|---|---|---|---|---|
| Fabric of the invention | 260 | 75 | 74 | 170 | 10,0 | 5 |
| Modacrylic / cotton | 260 | 25 | 25 | 126 | 4.3 | 4 |
| FR treated cotton | 340 | 28 | 29 | 139 | 9.1 | 3 |
| Aramid | 260 | 51 | 49 | 109 | 2.3 | 3-4 |

The fabric of the invention has a higher tear strength compared with most of the other materials on the market.

### Comfort testing: Results according to Table 3

### Alambeta - Heat penetration coefficient:

The fabric was tested for its comfort properties. The Alambeta test measures the rate of transmission of body heat through the fabric. Fabrics with a high heat penetration coefficient feel cooler and this makes them more comfortable to wear. Referring to the results of Table 3 the fabric of the invention shows the highest heat penetration coefficient, resulting in the coolest fabric touch.

### Short time water vapor absorption Fi:

The fabric was tested for short term water vapour absorption (Fi) according to EN ISO 31092 using the human skin model apparatus. A high water vapour absorbency indicates the fabric is capable of positively managing the moisture in its environment. This helps to keep the body dry and cool. Referring to the results of Table 3 the fabric of the invention shows the highest short time water vapor absorption, resulting in the best wearing comfort.

This can help to avoid the risk of heat stress and heat stroke and will improve the physiological performance of the wearer.

### Colour fastness testing:

Due to the usage of 100% spundyed fibres, or quality dyeing procedures high colour fastness can be achieved, as colours never wash or wear out.

### Example 2

The fabric of example 1 according to the invention was assessed subjectively and compared to commercially available fabrics used for Personal Protective Clothing. The results are given in Table 4, last column. In this table the scoring system is 1 to 3: 1 = poor, 3 = excellent.

In every parameter judged, the fabric of example 1 was given the highest possible score. No other fabric assessed achieved the same high level on assessment.

## Claims

1. A flame resistant fabric for use in personal protective clothing which provides a high level of protection from flames and other sources of heat such as molten metal splash and electric arc, which is made from an intimate blend of flame resistant cellulosic fibres with high temperature resistant polymer fibres and standard flammable synthetic fibres, wherein the intimate blend is in the form of a yarn, **characterized in that** the blend ratio of the yarn is
- from 65 to 90% flame resistant Modal fibres,
- from 10 to 20 % high temperature resistant polymer fibres and
- from 10 to 20% standard flammable synthetic fibres.

2. Fabric according to claim 1, wherein the blend ratio of the yarn is
- from 65 to 75% flame resistant Modal fibres,
- from 12,5 to 17,5% high temperature resistant polymer fibres and
- from 12,5 to 17,5% standard flammable synthetic fibres.

3. Fabric according to claim 1, wherein the flame resistant Modal fibres of the yarn are staple fibres with a staple length of between 75 and 90 mm.

4. Fabric according to claim 1, wherein the flame resistant Modal fibres of the yarn have been made flame resistant by addition of an FR agent during or after fibre production.

5. Fabric according to claim 1, wherein the high temperature resistant polymer fibres are chosen from the group consisting of para-aramid, meta-aramid, aromatic PES, PBI and blends of these fibres.

6. Fabric according to claim 1, wherein the standard flammable synthetic fibres are selected from the group including PA6, PA6.6 and PES fibres.

7. Fabric according to claim 1 which has been made antistatic by the addition of 1% to 5% of an antistatic staple fibre to the blend.

8. Fabric according to claim 1 which has been made antistatic by incorporating a grid pattern of yarns consisting of the intimate blended yarn twisted with antistatic continuous filament yarn.

9. Fabric according to any one of claims 1 to 8 which is produced by weaving or knitting.

## Patentansprüche

1. Flammbeständiger Stoff für den Einsatz im Bereich Persönliche Schutzbekleidung, der einen hohen Schutz vor Gefährdungen durch Flammen oder andere Hitzequellen, wie z. B. geschmolzene Metallspritzer und Störlichtbogen, welcher aus einer Intimmischung aus FR-Zellulosefasern mit hochtemperaturbeständigen Polymerfasern und synthetischen Standardfasern hergestellt ist, und bei dem die Intimmischung in Form eines Garns vorliegt, **dadurch gekennzeichnet, dass** das Mischungsverhältnis des Garnes vorzugsweise
- zwischen 65 und 90 % flammbeständige Modalfasern,
- zwischen 10 und 20 % hochtemperaturbeständigen Polymerfasern und
- zwischen 10 und 20 % entflammbaren synthetischen Standardfasern
liegt.

2. Stoff gemäß Anspruch 1, bei dem das Mischungsverhältnis des Garnes vorzugsweise
- zwischen 65 und 75 % FR-Zellulosefasern,
- zwischen 12,5 und 17,5 % hochtemperaturbeständigen Polymerfasern und
- zwischen 12,5 und 17,5 % entflammbaren synthetischen Standardfasern
liegt.

3. Stoff gemäß Anspruch 1 bei dem die flammbeständigen Modalfasern des Garnes Stapelfasern mit einer Stapellänge zwischen 75 und 90 mm sind.

4. Stoff gemäß Anspruch 1, bei dem die flammbeständigen Modalfasern des Garnes während oder nach der Faserherstellung durch den Zusatz eines FR-Wirkstoffes flammbeständig gemacht wurden.

5. Stoff gemäß Anspruch 1, bei dem die hochtemperaturbeständigen Polymerfasern aus der Gruppe bestehend aus Para-Aramid, Meta-Aramid, aromatischem PES, PBI und Mischungen dieser Fasern ausgewählt werden.

6. Stoff gemäß Anspruch 1, bei dem die entflammbaren synthetischen Standardfasern aus der Gruppe ausgewählt werden, zu der PA6-, PA6,6- und PES-Fasern gehören.

7. Stoff gemäß Anspruch 1, der durch Zusatz von 1 % bis 5 % antistatischer Stapelfaser zu der Mischung antistatisch gemacht wurde.

8. Stoff gemäß Anspruch 1, der durch Einschluss eines Rastermusters aus Garnen, die aus dem mit antistatischen Endlosfilamentgarnen verzwirnten Grundgarn bestehen, antistatisch gemacht wurde.

9. Stoff gemäß einem der Ansprüche 1 bis 8, der durch Weben oder Stricken produziert wurde.

## Revendications

1. Tissu résistant aux flammes, destiné à une utilisation dans le domaine des vêtements de protection personnelle, offrant une protection élevée contre les flammes ou autres sources de chaleur, comme des projections de métal en fusion et des arcs électriques, réalisé à partir d'un mélange Intime de fibres cellulosiques résistant aux flammes et de fibres de polymère résistant aux températures élevées, et de fibres synthétiques inflammables standard, et dans lequel le mélange intime est présent sous la forme d'un fil, **caractérisé en ce que** le rapport de mélange du fil est
- de 65 à 90 % de fibres Modal résistant aux flammes,
- de 10 à 20 % de fibres de polymère résistant aux températures élevées et
- de 10 à 20 % de fibres synthétiques inflammables standard.

2. Tissu selon la revendication 1, dans lequel le rapport de mélange du fil est
- de 65 à 75 % de fibres cellulosiques résistant aux flammes,
- de 12,5 à 17,5 % de fibres de polymère résistant aux températures élevées et
- de 12,5 à 17,5 % de fibres synthétiques inflammables standard.

3. Tissu selon la revendication 1, dans lequel les fibres Modal résistant aux flammes du fil sont des fibres discontinues dont la longueur est comprise entre 75 et 90 mm.

4. Tissu selon la revendication 1, dans lequel les fibres Modal résistant aux flammes du fil ont été rendues ininflammables pendant ou après la fabrication de la fibre, par l'adjonction d'une substance active résistant aux flammes.

5. Tissu selon la revendication 1, dans lequel les fibres de polymère résistant aux températures élevées sont choisies dans le groupe comprenant le para-aramide, le méta-aramide, le PES aromatique, le PBI et des mélanges de ces fibres.

6. Tissu selon la revendication 1, dans lequel les fibres synthétiques inflammables standard sont sélectionnées dans le groupe dont font partie les fibres PA6, PA6,6 et PES.

7. Tissu selon la revendication 1 qui a été rendu antistatique par l'adjonction, au mélange, de 1 % à 5 % d'une fibre discontinue antistatique.

8. Tissu selon la revendication 1 qui a été rendu antistatique par l'incorporation d'une trame de fils constituée du fil en mélange intime, torsadé avec du fil de filaments continus antistatiques.

9. Tissu selon l'une des revendications 1 à 8 produit par tissage ou tricotage.
